

S. E. DITTMAN.  
MATERIAL FOR BUILDING UP PRINTING PLATES.  
APPLICATION FILED DEC. 27, 1913.

1,119,498.

Patented Dec. 1, 1914.

Fig. 1.



Fig. 2.



Fig. 3.



Witnesses:

Harry S. Gaither  
Charles A. Poole.

by

Boyle + Crouner

Inventor  
Samuel E. Dittman.

Attest

# UNITED STATES PATENT OFFICE.

SAMUEL E. DITTMAN, OF NEW YORK, N. Y.

## MATERIAL FOR BUILDING UP PRINTING-PLATES.

1,119,498.

Specification of Letters Patent.

Patented Dec. 1, 1914.

Application filed December 27, 1913. Serial No. 303,961. &

*To all whom it may concern:*

Be it known that I, SAMUEL E. DITTMAN, a citizen of the United States, and a resident of New York, in the county of New York and State of New York, have invented certain new and useful Improvements in Material for Building Up Printing-Plates; and I do hereby declare that the following is a full, clear, and exact description thereof, reference being had to the accompanying drawings, and to the letters of reference marked thereon, which form a part of this specification.

This invention relates to an improved article of manufacture adapted for use in the art of printing and more particularly for building up forms in printing presses.

The process of building up printing plates or "leveling up" plates as it is often termed is one commonly used in the art of printing, and consists of treating the printing plate in such a manner that portions of the same, which are by tests found not to be at the required level for producing the proper impression, are brought to the proper level by applying patches of paper to the reverse face of the printing plate.

In the art of building up printing forms in the manner heretofore unknown to the art as illustrated and described, for instance, in Letters Patent of the United States granted to Frank J. Slader, No. 984,859, in which Letters Patent I have acquired certain rights and interest, a material such as soap or wax has been applied to the plate and the latter subjected to a pressure of the impression cylinder in excess of the degree of pressure required in the operation of printing. The soap or wax was crushed throughout the portions underlying the unduly high portions of the printing plate, thus spreading the material into the intervening spaces, and leaving the portions of the material underlying the relatively lower portions of the printing plate substantially unaltered or only crushed to such extent as to accomplish the necessary leveling required to properly build up the plate.

The material heretofore commonly used was in the form of numerous small disks of soap and like nonelastic materials readily susceptible to crushing. These disks were preferably laid at suitable distances apart between superimposed sheets of paper to assure the protection and retention of the said

disks. The operation of building up the plates was accomplished by depositing a number of these disks upon the back of the printing plate by means of a perforated plate, forming a die or mold for the disks, over which was scraped a bar of soap or wax. The disks deposited upon the plate remained after the removal of the perforated plate and a sheet was laid over the disks. The process is obviously commercially impractical as regards its application and use in the extensive and highly developed state of the printing art at the present day in that the large number of plates to be thus treated would result in a great loss of time and money in the preparation of the sheets for each individual operation. Furthermore, it would be impossible to manufacture a large quantity of these sheets by the above mentioned or any known method and thus maintain a constant supply at hand, for the reason that the normally soft condition of the disks would require their almost immediate use. It would be impracticable to place the sheets upon the market as an article of sale owing to their inability to withstand handling, storing or transportation such as a marketable product must undergo. Furthermore, the size of the sheets would depend upon the size of the perforated plate or die, hence in the treatment of large printing plates, the use of a very large die, or the repeated use of a single die, would in either case be an expensive and laborious operation.

The principal object of my invention is to provide a durable and improved article of manufacture to be used for the purpose hereinafter described, that may be economically produced in large quantities; that may be bought and sold in commercial quantities upon the market, and that will not deteriorate or be susceptible to injury during shipment, or long periods of time occasioned by storage prior to use. To accomplish this end, I propose to produce an article of manufacture suitable for building up plates, in which the material adapted to be compressed to accomplish the proper treatment of the plates, shall be composed of a material which is normally sufficiently hard or non-compressible to withstand the normal pressure to which it is subjected in the operation of printing without being crushed or distorted to an extent which will affect the quality of the work, but capable of be-

ing softened or rendered more plastic, just prior to its use, by the application of a liquid agent, or in any other desirable manner, and which will reharden subsequent to the process of building up the printing plate.

5 My invention, therefore, consists in the matters hereinafter described, more particularly pointed out in the appended claims, and fully illustrated in the accompanying drawings in which,

10 Figure 1 is a view in perspective showing my proposed construction for the article of manufacture embodying my invention; Fig. 2 is a cross-sectional view taken on line 2—2, of Fig. 1, showing a sheet of the building up material applied to a printing plate. Fig. 3 is a cross-sectional view of a modified form of the building up material applied to a printing plate.

15 Referring to the drawings: The article of manufacture embodying my invention, as herein illustrated and described, comprises a sheet A, of paper or other suitable flexible or fibrous material of suitable thickness and quality, upon the surface of which are placed a plurality of cakes or disks C, each formed of a material which is by preference normally sufficiently hard, strong and rigid to withstand the pressure to which it is subjected in the operation of printing and which is adapted to be softened or rendered more plastic or compressible by means of a suitable solvent or other agent to enable the disks to be compressed while in a softened 20 or relatively plastic condition so as to compensate for irregularities in the surface of the printing plate. The disks are of uniform thickness and are arranged in any manner desired without regard to regularity, but spaced apart at sufficient distances to provide, in effect, a layer of material of uniform thickness.

25 The material of which I propose to make the disks C, by preference, embodies a combination of substances, having such qualities as are adapted to render the disks sufficiently hard to resist the tendency to become crushed or distorted by handling in shipment or storage or in the operation of printing as already suggested, to be capable of being softened by the application of a suitable agent, thus being susceptible to compression by the normal pressure of the impression cylinder of a printing press when in such softened condition, and to resume its normal degree of hardness after the disks have been crushed. A material having these qualities and which has been found in practice to be satisfactory 30 for the purpose of this invention consists of a composition of glue sixty-one per cent. (61%), wheat flour thirty-one per cent. (31%), and glycerin eight per cent. (8%), or a composition of talcum powder forty- 35 seven per cent. (47%), dextrin, twelve

per cent. (12%), starch, five per cent. (5%), water, twenty-six per cent. (26%), calcium chlorid two per cent. (2%), glucose six per cent. (6%), formaldehyde two per cent. (2%), combined in the proportions indicated to obtain the desired degree of hardness or rigidity and strength and the desired degree of compressibility and plasticity for accomplishing the purposes of the invention.

40 As a preferable construction of my improved building up material, I propose to apply the disks to the sheet of paper by means of its own adhesive qualities or in any suitable manner such as will insure the close adherence of the disks thereto.

45 The sheets to which the disks are applied may be of any desirable size as, for instance, a continuous sheet having the form of a roll of paper or other suitable flexible or fibrous material to which the disks are applied in any convenient manner. I prefer, however, to employ mechanical means for applying the disks to the paper, such mechanical means embodying, for instance, a device adapted to form the disks from an adequate supply of the composition and to apply the same to sheets or to a roll of paper constantly fed to the device. In this manner it is possible to manufacture large quantities of the material. As hereinbefore suggested, 50 the disks are normally in a hardened condition, which condition they would assume substantially at the time of application to the paper.

55 The "building up" sheets, as they may be called, which comprise the hardened disks securely affixed to the paper, are obviously capable of being shipped or handled without the liability of injury; thus large quantities may be manufactured and put on the market in convenient form, as, for instance, in rolls or packages of any desired number of single sheets.

60 To render the sheets suitable for use it is necessary that the disks be softened in order that they be readily susceptible to compressing during the operation of leveling up of a plate. For this purpose a suitable agent is employed as for instance, water. This agent may be applied in any convenient manner as by dipping the sheets in the liquid or solvent or spraying by means of an atomizer. The softening operation is perfectly carried out just prior to the application of the sheet to the printing plate, 65 requiring the treatment hereinbefore set forth and pressure sufficient to compress the disks while in a softened or plastic condition so as to cause the material of which the disks are formed to conform to or compensate for the irregularities in the thickness of the printing plate or the surfaces of the same in such a manner as to render the printing surface uniform. The material of which the disks or building up material is 70

formed being then allowed to harden so as to withstand pressure applied in the operation of printing.

The operation of subjecting a printing plate to treatment with my improved form of building up material, consists primarily in securing a sheet corresponding in size to that of the plate, which may be cut from a roll or a large sheet of the material, in the instance that such be the form of the supply at hand. The disks are then softened in the manner before indicated, and the sheet is applied, as shown in Fig. 2, to the reverse side of the plate D, having a cut or printing characters of any desired kind upon its front or printing face, not shown, said sheet being preferably applied with the disks D, in contact with the reverse side of the printing plate, and preferably secured thereto by their own adhesive qualities. This plate with its backing of building up material upon its reverse face is then placed in position in the printing press, and upon passing it under the impression roller, the pressure exerted by the same will level up the plate by variously compressing the disks under the portions of the plate that are slightly above the desired printing level. In this manner the entire printing surface of the plate is rendered uniform or reduced to a uniform height corresponding to the desired printing level of the press. It is desirable that the pressure upon the plate and the leveling up sheet be sufficient to compress all of the disks to such an extent to compensate for any irregularities in the surface of the printing plate. For this reason it is desirable that the thickness of the sheet and disks be slightly in excess of the height to which the most depressed points in the cut or printing plate are required to be leveled, so that all of the disks will be, by preference, more or less compressed by the pressure of the impression cylinder. The printing plate having been leveled up by the compressing of the disks in the manner described, it is allowed to stand for a short interval during which time the liquid softening agent will be evaporated and the disks will again become hardened to their original condition. The printing plate may now be used for the purpose of reproducing printed copies therefrom.

One of the advantages of using this improved form of building up material, lies in the fact that the material before being subjected to the pressure of the impression cylinder may be softened to such a degree as to be readily compressible by the normal printing pressure of the impression cylinder, whereas in the process heretofore used, a pressure greater than the normal printing pressure of the impression cylinder was required to crush the disks of soap or wax in that such materials maintained a constant

degree of plasticity. In this manner the necessity of applying a pressure greater than the normal is eliminated. Furthermore, the use of disks composed of material which rehardens subsequent to the process of softening the disks and the leveling of the printing plate, produces a backing for the plate much better suited to withstand long usage and handling of the printing plate, and the pressure of the impression cylinder in the printing operation, whereas, soap, wax, paper or the like materials incapable of being softened in the manner described are not suitable as a medium for withstanding excessive handling and pressures and which are known to be susceptible to variations of working conditions as for instance of temperature or humidity.

The application of a second sheet B, may be included in the manufacture of the building up material, thus providing additional means for protecting the disks from injury occasioned by packing, shipping and storing. In the manufacture of a building up material consisting of disks interposed between two sheets of paper, the sheet B, Fig. 3, would be applied subsequently to the application of the disks to the sheet A, and in such manner as to adhere to the surfaces of said disks.

It is to be understood that any material such as cloth may be substituted for paper in the manufacture of my improved building up sheets, and that any desired quality of material may be used.

In view of the fact that several materials may be utilized in the production of an article embodying the features of my invention, I do not wish to be limited to the material or composition described, except so far as set forth in the appended claims.

I claim as my invention:

1. In the art of printing, a material adapted to be applied to the reverse face of a printing plate for leveling or building up the same, comprising a sheet of paper and a plurality of cakes secured to said sheet, said cakes being composed of a material normally non-compressible under the printing pressures, and adapted to be softened to render them compressible during the leveling or building up process.

2. In the art of printing, a material adapted to be applied to the reverse face of a printing plate for leveling or building up the same, comprising a sheet of paper and a plurality of disks, secured in spaced relation to said sheet, said disks being composed of a material normally non-compressible under the printing pressures and adapted to be softened by the application of a softening agent to render them compressible under the normal printing pressure during the leveling or building up process.

3. In the art of printing, a material

adapted to be applied to the reverse face of a printing plate for leveling or building up the same, comprising superimposed sheets of paper and a plurality of disks interposed between said sheets, said disks being composed of a material normally non-compressible under the printing pressures, and adapted to be softened to render them compressible during the leveling or building up process.

4. An article of manufacture adapted to be used for leveling or building up printing plates, comprising a sheet of flexible material and a plurality of disks secured to said sheet, and consisting of a material comprising glue, flour and glycerin.

5. An article of manufacture, adapted to

be used for building up printing plates, comprising a sheet of paper, a plurality of disks secured to the sheet and consisting of 20 a material containing sixty-one per cent. (61%) of glue, thirty-one per cent. (31%) of wheat flour and eight per cent. (8%) of glycerin, said disks being adapted to be treated with water to render them compressible.

In testimony, that I claim the foregoing as my invention I affix my signature in the presence of two witnesses, this 15th day of December A. D. 1913.

SAMUEL E. DITTMAN.

Witnesses:

ELWOOD W. BAKER,  
NELLIE H. EFROS.